

[54] **ELECTROLESS GOLD PLATING ON  
REFRACTORY METALS**[75] Inventor: **Richard Kent Trueblood, Leucadia,  
Calif.**[73] Assignee: **Ceramic Systems, San Diego, Calif.**[22] Filed: **June 8, 1973**[21] Appl. No.: **368,431**[52] **U.S. Cl.** **117/50, 106/1, 117/130 E,  
117/160 R**[51] **Int. Cl.** **C23c 3/02**[58] **Field of Search** **117/50, 47 R, 130 E, 160 R,  
117/213, 35 S; 106/1; 29/199; 204/46, 38 B**[56] **References Cited****UNITED STATES PATENTS**

|           |         |               |           |
|-----------|---------|---------------|-----------|
| 3,032,436 | 5/1962  | Gostin et al. | 117/130 E |
| 3,212,918 | 10/1965 | Tsu et al.    | 117/35 S  |
| 3,230,098 | 1/1966  | Robinson      | 106/1     |

|           |         |                          |           |
|-----------|---------|--------------------------|-----------|
| 3,396,042 | 8/1968  | Duva.....                | 106/1     |
| 3,468,676 | 9/1969  | Schneble, Jr. et al..... | 117/130 E |
| 3,589,916 | 6/1971  | McCormack .....          | 106/1     |
| 3,627,558 | 12/1971 | Roger et al. ....        | 117/50    |
| 3,672,939 | 6/1972  | Miller .....             | 117/35 S  |

*Primary Examiner*—Charles E. Van Horn*Assistant Examiner*—Michael W. Ball*Attorney, Agent, or Firm*—Ronald E. Grubman[57] **ABSTRACT**

For the electroless gold plating of metals, including refractory metals such as molybdenum, tungsten, columbium, and cobalt, a process is provided which includes activating the metal with an alkaline descaler followed by a dilute acid, and immersing the metal in a plating bath which is composed of a soluble gold salt, an organic chelating compound, a non-ammoniacal organic buffering and complexing agent, and a non-ammoniacal alkali hydroxide.

**6 Claims, No Drawings**

## ELECTROLESS GOLD PLATING ON REFRACTORY METALS

### BACKGROUND AND SUMMARY OF THE INVENTION

This invention relates to improvements in the process of electroless depositing of soft, ductile gold on metals, and particularly on refractory metals by which we mean, for example, such metals as molybdenum, tungsten, columbium, and cobalt. Heretofore, electroless depositing of gold on refractory metals has been difficult. Among the electroless plating process known in the prior art, plating solutions are used which include an organic chelating agent and an ammonium buffering agent. The ammonium buffering agent serves the dual purposes of regulating the pH of the bath and exerting a complexing action to complex some of the replaced metal ions from the surface of the metal being plated. When used to plate refractory metals such as molybdenum, tungsten, columbium, or cobalt, however, solutions of this kind could only deposit pure gold to thicknesses of a few microinches. The deposits obtained were of coarse texture, dark orange to brown in color, mottled in appearance, uneven in distribution, and lacking in adherence. These problems have rendered the heretofore available electroless gold solutions completely unsatisfactory for depositing gold films on refractory metals such as the metals mentioned above.

It is therefore the object of this invention to provide an electroless plating process capable of providing pure, soft, ductile gold of uniform yellow appearance to any desired thickness up to approximately 200 microinches, on metal substrates including substrates of the metals molybdenum, tungsten, columbium, and cobalt, or on previously plated gold substrates.

The present invention achieves this object by providing a plating bath composed of a soluble gold salt such as the double cyanide of an alkali metal (e.g. potassium gold cyanide), an organic chelating compound (e.g. the tetra sodium salt of ethylenediaminetetraacetic acid tetrahydrate), a non-ammoniacal organic buffering and complexing agent (e.g. sodium potassium tartrate, "Rochelle Salt"), and a non-ammoniacal alkali hydroxide (e.g. sodium hydroxide). In the aforementioned bath, the soluble gold salt serves as a source of gold ions. The organic chelating compound serves to tie-up, or chelate, some of the undesirable metal ions which would otherwise contaminate the plating bath. These undesirable metal ions may be introduced into the bath as impurities in the plating chemicals, as reaction products during the plating process, or by accidental contamination through "drag-in" following cleaning and activation prior to the plating process. The alkali hydroxide serves to establish the range of pH necessary for operation of the bath, and the organic buffering and complexing agent serves to regulate the pH of the bath within the established range. To achieve good plating results, the above-described plating bath is used to plate metals which have first undergone an activating sequence which includes immersion of the metals in an alkaline descaler followed by an acid rinse. This procedure provides a suitable surface for the subsequent plating.

The present invention may be used whenever and wherever a gold protective layer on metals is desired or required. The invention has a potentially wide application in the fields of electronics, wherein powders of the

refractory metals are sintered to ceramic insulators and subsequently gold plated to allow their brazing to metal members. Sintered metal powders are also used in hybrid microelectronics wherein these powders are overplated with gold and act as electrical conductors on ceramic substrates. This invention would be of incalculable value as an overplating for these sintered metal powders in that it would allow extremely uniform plating over all metallized areas.

### DESCRIPTION OF THE PREFERRED EMBODIMENT

In accordance with the preferred embodiment, the metal to be plated is first subjected to an activating treatment in preparation for immersion in a plating bath. The activating, or cleaning process includes first soaking the metal in a hot alkaline descaler (e.g. Iso-prep 180 manufactured by Allied Kelite Products Inc.) at a temperature of between 80°C and 100°C. The metal is then rinsed in deionized water, and further rinsed in a hot dilute acid solution (e.g. a 20-50% hydrochloric acid solution) at a temperature of between 80°C and 100°C. A final rinse is performed using boiling deionized water.

After the metal to be plated has undergone the above-described activation treatment, it is immersed in a plating bath which includes a soluble gold salt (e.g. potassium gold cyanide) present in amounts ranging from 2 to 10 grams per liter with 4-5 grams per liter preferred, which serves as the source of supply for gold ions. Other soluble gold salts may be also used (e.g. sodium gold cyanide) but the potassium salt is preferred and more commercially available.

An organic chelating compound (e.g. tetra sodium ethylenediaminetetraacetate tetrahydrate) is present in amounts ranging from 10-50 grams per liter, with 20 grams per liter being preferred, and serves to tie-up or chelate undesirable metal ions which may be introduced into the bath. Other chelating compounds may also be used (e.g. ethylenediamine or triethylanolamine) but tetra sodium ethylenediaminetetraacetate tetrahydrate is preferred and readily available.

A non-ammoniacal organic buffering and complexing agent, for example an alkali metal salt of a weak acid such as sodium potassium tartrate, is present in amounts ranging from 25-100 grams per liter, with 55-70 grams per liter being preferred, and serves to regulate the bath pH to maintain the proper range for best plating efficiency. Increasing the amount of buffering and complexing agent decreases the rate of gold deposition but produces a finer-grained and brighter deposit. Decreasing the amount of buffering and complexing agent increases the gold deposition rate but leads to a coarse-grained slightly orange deposit. Other non-ammoniacal buffering and complexing agents may be used (e.g. sodium or potassium citrate) but "Rochelle Salt," sodium potassium tartrate, is preferred.

A non-ammoniacal alkali hydroxide (e.g. sodium hydroxide) is present in amounts ranging from 5 to 50 grams per liter, with 8-18 grams per liter being preferred, and serves to establish the pH necessary for operation of the bath. Increasing the amount of the alkali hydroxide increases the gold deposition rate but oxidizes the metal substrate through chemical attack and leads to poor plating adherence on molybdenum, columbium, and tungsten. Oxidation is not as critical a

problem when plating cobalt, and a higher alkali hydroxide concentration is desirable, 30 grams per liter being preferred. Other nonammoniacal alkali hydroxides may be used (e.g. potassium hydroxide) but sodium hydroxide is preferred. Under no conditions should ammonium hydroxide or the salts thereof be added in place of or in addition to the alkali hydroxides. Doing so "poisons" the bath so that the rate of gold deposition is greatly reduced if not halted altogether.

The following are examples of electroless plating processes according to the invention, based on one liter of plating solution:

Example 1

|                                                       | Grams/Liter |
|-------------------------------------------------------|-------------|
| Potassium gold cyanide                                | 4           |
| Tetra sodium ethylenediaminetetraacetate tetrahydrate | 20          |
| Sodium potassium tartrate                             | 58          |
| Sodium hydroxide                                      | 18          |
| Deionized water                                       | Remainder   |

The pH of the bath was 13.2-13.5. The bath was used to plate tungsten metallized ceramic circuit boards after first undergoing the following cleaning sequence:

|                                     |         |
|-------------------------------------|---------|
| Alkaline descaler at 95°C           | 15 min. |
| Deionized water rinse               | 1 min.  |
| 20% hydrochloric acid rinse at 85°C | 5 min.  |
| Deionized water rinse at 100°C      | 5 min.  |

The circuit boards were then immersed in a beaker of the plating solution and remained there at 100°C for 35 minutes. On removing the circuit boards from the bath and subsequently rinsing and drying, the thickness of gold deposited, as determined by the Weight-Area Method, was approximately 120 microinches.

Example 2

|                                                       | Grams/Liter |
|-------------------------------------------------------|-------------|
| Potassium gold cyanide                                | 4           |
| Tetra sodium ethylenediaminetetraacetate tetrahydrate | 20          |
| Sodium potassium tartrate                             | 58          |
| Sodium hydroxide                                      | 30          |
| Deionized water                                       | Remainder   |

The pH of the bath was 13.4-13.7. The bath was used to plate tungsten metallized ceramic circuit boards which had been given an electroless cobalt overplate of approximately 40 microinches thickness. After the circuit boards had been removed from the cobalt plating bath, they were subjected to the cleaning sequence of example 1 above and transferred to the above gold plating bath. The circuit boards remained in the bath at 100°C for 45 minutes. On removing the circuit boards from the bath and subsequently rinsing and drying, the thickness of gold deposited, as determined by the Weight-Area Method, was approximately 100 microinches.

Example 3

|                                                       | Grams/Liter |
|-------------------------------------------------------|-------------|
| Potassium gold cyanide                                | 2           |
| Tetra sodium ethylenediaminetetraacetate tetrahydrate | 20          |
| Sodium potassium tartrate                             | 70          |

Example 3-Continued

|                  |           |
|------------------|-----------|
| Sodium hydroxide | 8         |
| Deionized water  | Remainder |

5 The pH of the bath was 13.0-13.2. The bath was used to plate columbium metal plates after first undergoing the cleaning sequence of Example 1 above.

10 The columbium plates were allowed to remain in the solution for 15 minutes at 100°C. Upon their removal from the bath and after subsequent rinsing and drying, the thickness of gold deposited, as determined by the Weight-Area Method, was approximately 200 microinches.

Example 4

|                                                       | Grams/Liter |
|-------------------------------------------------------|-------------|
| Potassium gold cyanide                                | 4           |
| Tetra sodium ethylenediaminetetraacetate tetrahydrate | 20          |
| Sodium potassium tartrate                             | 58          |
| Sodium hydroxide                                      | 18          |
| Deionized water                                       | Remainder   |

25 The pH of the bath was 13.2-13.5. The bath was used to plate molybdenum metal plates after first undergoing the cleaning sequence of Example 1 above. The molybdenum plates were allowed to remain in the solution for 30 minutes at 100°C (boiling). Upon their removal from the bath and after subsequent rinsing and drying, the thickness of gold deposited, as determined by the Weight-Area Method, was approximately 55 microinches.

30 Although the plating baths in the above examples were operated at the boiling point (approximately 100°C), temperatures as low as 80°C result in satisfactory deposits. Operation at the boiling point has the advantage, however, of providing continuous bath agitation by virtue of the boiling point action, thereby increasing the deposition rate. Thus, less time is required to obtain equivalent deposition thickness when the process is operated at the boiling point.

35 In the above examples, the gold deposits obtained had the yellow-color of pure gold and were of 24 karat purity.

40 I claim:

45 1. A method for plating refractory metals comprising the steps of:

50 activating the metal to be plated by immersing it in an alkaline descaler at a temperature in the range of 80°-100°C, rinsing the metal in deionized water, rinsing the metal in a dilute acid at a temperature in the range of 80°-100°C, and rinsing the metal in boiling deionized water; and

55 immersing the metal in an electroless gold plating bath consisting essentially of water, about 2 to 10 grams per liter of a soluble gold salt selected from the group consisting of potassium gold cyanide and sodium gold cyanide, about 10 to 50 grams per liter of an organic chelating compound, about 25 to 100 grams per liter of a non-ammoniacal alkali metal salt of a weak acid to serve as a buffering and complexing agent, and a non-ammoniacal alkali metal hydroxide in an amount sufficient to bring the pH of the bath to between about 13 to 14.

60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030

the metal in a hydrochloric acid solution in the range of 20-50 vol. percent.

3. A method as in claim 1 wherein the step of immersing the metal in an electroless gold plating bath including a non-ammoniacal alkali metal salt of a weak acid comprises the step of immersing the metal in an electroless gold plating bath including a non-ammoniacal alkali metal salt of a weak acid selected from the group consisting of sodium potassium tartrate, sodium citrate, and potassium citrate.

4. A method as in claim 1 wherein the step of immersing the metal in an electroless gold plating bath including a non-ammoniacal alkali metal hydroxide comprises the step of immersing the metal in an electroless gold plating bath including a non-ammoniacal alkali metal hydroxide selected from the group consisting of

sodium hydroxide and potassium hydroxide.

5. A method as in claim 1 wherein the step of immersing the metal in an electroless gold plating bath including an organic chelating compound comprises the step of immersing the metal in an electroless gold plating bath including an organic chelating compound selected from the group consisting of tetra sodium ethylenediaminetetraacetate tetrahydrate, ethylenediamine, and triethanolamine.

10 6. A method as in claim 1 wherein the step of immersing the metal in an electroless gold plating bath comprises the step of immersing the metal in an electroless gold plating bath whose temperature is the boiling point temperature of said bath.

\* \* \* \* \*

20

25

30

35

40

45

50

55

60

65

UNITED STATES PATENT OFFICE  
CERTIFICATE OF CORRECTION

Patent No. 3,862,850 Dated January 28, 1975

Inventor(s) Richard Kent Trueblood

It is certified that error appears in the above-identified patent and that said Letters Patent are hereby corrected as shown below:

Column 1, line 12, cancel "process" and substitute  
-- processes --; line 34, cancel "molybenum" and substitute  
-- molybdenum --; and

Column 4, line 65, cancel "to", second occurrence, and  
substitute -- and --.

Signed and sealed this 8th day of April 1975.

(SEAL)

Attest:

RUTH C. MASON  
Attesting Officer

C. MARSHALL DANN  
Commissioner of Patents  
and Trademarks